

## UNITED STATES PATENT OFFICE

CHARLES BOULANGER, OF CLICHY, FRANCE, ASSIGNOR TO SOCIETE CONTINENTALE PARKER, OF CLICHY, FRANCE

PROCESS AND PRODUCT FOR PROTECTING ALUMINIUM, MAGNESIUM AND THEIR ALLOYS AGAINST CORROSION

No Drawing. Application filed October 21, 1929, Serial No. 401,384, and in France November 10, 1928.

The present invention has for its object a process of protecting the surface of aluminium, magnesium, or their alloys, against attacks by salt solutions, such as chloride of sodium, or by moist air loaded with particles of these solutions, for instance sea air capable of causing the alteration or corrosion of the metal.

The process is essentially characterized by the fact that, by means of a salt bath, a protecting deposit is formed at the surface of the metal, and that, to form this deposit, use is made of solutions of alkali metal salts such as chromates, vanadates, molybdates, tungstates, titanates, uranates, niobates, manganates, etc., either alone, or mixed together.

It is necessary that the metal chosen can give at least two oxides, the most oxygenated of which gives an alkali salt soluble in an alkaline solution. By reduction, the corresponding oxide is brought back to the state of sub-oxide. Thus, a manganate corresponding to managanic acid  $MnO_3H_2O$ , will be brought back to the state of  $Mn_2O_3$  or of  $Mn_3O_4$ , which are stable, do not corrode when in use, and form at the surface of aluminium, for instance, the desired protecting layer.

The formation of this layer can be obtained by immersion of the metal part or member in a bath of the chosen salt, at a suitable degree of concentration and at a suitable temperature. The bath must be rendered alkaline by the addition of an alkali carbonate, or of the corresponding alkali hydroxide.

For instance for protecting an article made of aluminium, it can be immersed in a boiling solution of carbonate of sodium at about 1%, and of molybdate of sodium or potassium at 0.5%.

It has been found that the following process, derived from the preceding one, procures special advantages concerning the practical industrial carrying out of the process.

A better preservation of these salts in presence of moisture can be obtained by addition of a small quantity of a salt, such as borate of soda, which is without action on the deposited oxide film and on the metal to be protected.

A mixture of these two salts gives, in accordance with the present invention, the base product suitable for the preparation of the protecting bath. A proper proportion is that comprising 1 part of alkali sulpho-molybdate and 5 parts of alkali phospho-chromate. 55

It is to be understood that these proportions are not limitative; they simply constitute an example, since use can be made of sulpho-tungstate instead of sulpho-molybdate, or of sulpho-uranate, with phospho-vanadate or phospho-manganate, either alone or mixed together. 60

By way of example, the following proportions can be indicated for protecting aluminium: 65

Mixture of phospho-chromate and of sulpho-molybdate of potash—0.5% of the bath.

Carbonate of Solvay soda: 1% of the solution. 70

The concentration of the solution in alkali carbonate varies but slightly in use. The loss of salt caused by deposition, will be compensated by the introduction of a further quantity of salt in proportion as the bath will 75 become weaker.

The above mentioned salts are stable, they do not alter under the action of air and moisture, they are extremely soluble. The mixing of these salts with carbonate of soda procures the same qualities of unalterableness and of solubility. 80

The treatment of the article to be protected is effected at boiling point; the duration of the treatment depends on the thickness of the deposit it is desired to obtain. 85

The protecting layer constitutes an excellent holding surface for any varnish, paint, fatty bodies, enamels, etc.

Claims:

1. Process for protecting articles made of aluminium, magnesium, or their alloys, against corrosion, comprising the treatment of the said articles in a bath containing carbonate of soda and an alkali salt of the most oxygenated oxide of a metal capable of forming at least two oxides the most oxygenated one being soluble in alkaline solution and the less oxygenated one being insoluble. 95
2. Process for protecting articles made of 100

aluminium, magnesium, or their alloys, against corrosion, comprising the treatment of the said articles in a bath containing carbonate of soda and a mixture of alkali sulpho-molybdate and alkali phospho-chromate.

3. Process for protecting articles made of aluminium, magnesium, or their alloys, against corrosion, comprising the treatment of the said articles in a bath containing carbonate of soda and a mixture composed of 1 part of alkali sulpho-molybdate and 5 parts of alkali phospho-chromate.

10 4. Product serving to produce a protecting layer on articles made of aluminium, magnesium or their alloys, comprising a carbonate of alkali metal and a salt formed by an alkali metal and by one of the following metals; vanadium, molybdenum, tungsten, titanium, uranium, niobium, manganese and chrome-

20 5. Process for protecting articles made of aluminium, magnesium, or their alloys, comprising the treatment of the said articles in a bath, containing carbonate of soda and an alkali salt of a metal capable of giving at least two oxides, such as vanadium, molybdenum, tungsten, titanium, uranium, niobium, manganese and chromium.

25 In testimony whereof I have hereunto  
30 affixed my signature.

CHARLES BOULANGER.

35

40

45

50

55

60